

# United States Patent [19]

Mamantov

[11] Patent Number: 4,802,970

[45] Date of Patent: Feb. 7, 1989

[54] PROCESS FOR PREPARING FLUORINE BY  
ELECTROLYSIS OF CALCIUM FLUORIDE

[75] Inventor: Gleb Mamantov, Knoxville, Tenn.

[73] Assignee: E. I. Du Pont de Nemours and  
Company, Wilmington, Del.

[21] Appl. No.: 200,093

[22] Filed: May 31, 1988

[51] Int. Cl.<sup>4</sup> ..... C25B 1/00

[52] U.S. Cl. ..... 204/60

[58] Field of Search ..... 204/60

[56]

## References Cited

### U.S. PATENT DOCUMENTS

3,196,091 7/1965 Mastrangelo ..... 204/60  
3,324,016 6/1967 Langer ..... 204/60

Primary Examiner—G. R. Andrews

Attorney, Agent, or Firm—Charles E. Krukiel

[57]

## ABSTRACT

A process for producing fluorine from calcium fluoride in which calcium fluoride is dissolved in a molten salt electrolyte containing an alkali metal tetrafluoroborate and the melt is electrolyzed at a temperature below 400° C.

6 Claims, 1 Drawing Sheet





## PROCESS FOR PREPARING FLUORINE BY ELECTROLYSIS OF CALCIUM FLUORIDE

### BACKGROUND OF THE INVENTION

The present invention relates to an improved process for preparing fluorine by electrolysis of calcium fluoride ( $\text{CaF}_2$ ), and, more particularly, to a process in which fluorine is produced by dissolving  $\text{CaF}_2$  in a molten salt which contains an alkali metal tetrafluoroborate and electrolyzing the melt at a temperature below 400° C.

Fluorine is the most reactive of all known chemical elements, and it is prepared commercially by the electrolysis of hydrogen fluoride (HF). HF is prepared by reacting  $\text{CaF}_2$ , a naturally occurring mineral known as fluorspar, with sulfuric acid. During the electrolysis,  $\text{F}_2$  is produced at the anode, and  $\text{H}_2$ , which is vented and burned, is produced at the cathode. It would be desirable, therefore, to be able to produce fluorine directly from  $\text{CaF}_2$  and thereby eliminate the intermediate production of HF and the venting and burning of  $\text{H}_2$ .

U.S. Pat. No. 3,684,667 describes a method for producing fluorine and volatile fluorine compounds by the electrolysis of an electrolyte consisting of molten fluorides, e.g., calcium fluoride, using a plasma as the anode. The energy required to maintain a plasma is relatively high and can be expensive.

U.S. Pat. Nos. 3,196,090 and 3,196,091 describe the electrolysis of sodium tetrafluoroborate ( $\text{NaBF}_4$ ) at about 440° to 480° C. between a lead cathode and a graphite or gold anode. A fluorine/BF<sub>3</sub> mixture is produced at the anode, and a lead/sodium alloy is produced at the cathode. The  $\text{NaBF}_4$  starting material, however, is derived from HF as an intermediate.

Other attempts to produce fluorine directly from the electrolysis of  $\text{CaF}_2$  have been unsuccessful and have resulted instead in the production of fluorocarbons. For example, British patent No. 863,635 describes the electrolysis of  $\text{CaF}_2$  at 1450° C. using a carbon anode to produce CF<sub>4</sub>; British patent No. 863,602 describes the electrolysis of a mixture consisting of NaF,  $\text{CaF}_2$ , and MgF<sub>2</sub> to produce C<sub>1</sub> to C<sub>3</sub> fluorocarbons; and U.S. Pat. No. 2,835,711 describes the electrolysis of carbon with  $\text{CaF}_2$  and group IIA metal chlorides at temperatures of from 2000° to 5000° C. to produce fluorocarbons and chlorofluorocarbons.

### SUMMARY OF THE INVENTION

According to the present invention, a process has been developed for producing fluorine directly from  $\text{CaF}_2$  having the following steps:

(a) dissolving  $\text{CaF}_2$  in a molten salt electrolyte containing an alkali metal tetrafluoroborate; and

(b) electrolyzing the electrolyte at a temperature below 400° C. between an anode selected from a carbon material and nickel and a cathode selected from lead, tin, zinc and tin/zinc alloy.

A mixture of elemental fluorine and BF<sub>3</sub> is produced at the anode and calcium is deposited at the cathode along with the alkali metal of the tetrafluoroborate selected for the electrolyte. Optionally, the alkali metal tetrafluoroborate electrolyte may also contain one or more alkali metal fluorides or mixtures thereof. The alkali metals which are useful in the process of this invention are selected from Na, K and Li.

### BRIEF DESCRIPTION OF THE DRAWING

FIG. 1 is a cross sectional view of a typical electrolytic cell which can be used in practicing the process of this invention.

### DETAILED DESCRIPTION OF THE INVENTION

The present invention is an improved process for producing fluorine directly from  $\text{CaF}_2$  by electrolysis.

Referring now to FIG. 1 there is shown for purposes of illustration a cross-sectional view of an electrolytic cell of the type useful in practicing the process of this invention. The cell has a cylindrical flanged body 10 and a lid 12 typically fabricated from nickel. The lid is attached to the flanged body with bolts 14, and an o-ring, such as a "Viton" o-ring, 16 is placed between the mating flange surfaces as shown to seal the cell. A support ring 18 is provided, above which are located a series of cooling coils 20 for controlling the temperature of the upper portion of the cell. Two nested crucibles 22A and 22B made of alumina are located within the cell, the outer crucible 22A being a precautionary measure should the inner crucible 22B break or develop a leak during operation.

The cathode material, which forms a pool 24 beneath the molten electrolyte 26 during operation, is selected from analytical grades of Pb, Sn, Zn, and Sn/Zn alloy. The material to be used is washed successively with 1 M HCl,  $\text{H}_2\text{O}$ , and ethanol, then dried and molten in a ceramic crucible in an inert atmosphere, such as argon. The cathode material is then cooled and cut into pieces of appropriate size to be added to the cell. Sn/Zn alloys (e.g. 80/20 mol %) can be made by melting the corresponding amounts of Sn and Zn together in a ceramic crucible, cooling, and then cutting the alloy into the desired shape and size for introduction into the cell. Electrical contact with the cathode metal pool 24 can be made as shown using an alumina-sheathed  $\frac{1}{8}$  inch diameter (0.32 cm) nickel contact rod 28.

The anode 30 can be fabricated from different carbon materials, such as, for example, glassy carbon and pyrolytic graphite which are commercially available, or it can be fabricated from nickel. The preferred anode material is pyrolytic graphite for its availability, resistance to fluorine attack during cell operation, and price relative to other materials. In one example of this invention the anode material is pyrolytic graphite which has been machined into pieces 5 cm  $\times$  1.5 cm  $\times$  0.6 cm and is then degassed at 500° C. to remove impurities, especially water. Any convenient means can be used to secure the anode material to the anode contact lead 32. The contact lead, made of nickel, is insulated from the cell by an alumina sleeve.

The electrolytes comprise alkali metal tetrafluoroborates and may optionally include alkali metal fluorides, or mixtures thereof, in which the alkali metal is selected from K, Na and Li. Anhydrous KF (Aldrich, 99%), NaF (Aldrich, 99%), LiF (Alfa Products, 99%), NaBF<sub>4</sub> (Alfa Products, 99%), and LiBF<sub>4</sub> (Aldrich, 98%) were selected to demonstrate the process and are the preferred electrolyte components. Three tetrafluoroborate-containing electrolyte mixtures were prepared having the following compositions: LiBF<sub>4</sub>/LiF, 90/10 mol %; LiBF<sub>4</sub>/NaBF<sub>4</sub>, 50/50 mol %; and NaBF<sub>4</sub>/KF, 90/10 mol %. These mixtures were selected for their low melting points which, in turn, will reduce attack of the anode and cell by fluorine gener-

ated during operation. Other mixtures can also work satisfactorily.

The electrolyte components were prepurified by heating under vacuum at 200° C. for three days to remove as much water and HF as possible before being introduced into the cell. CaF<sub>2</sub> (Cerac, 99.99% anhydrous) was used without further purification.

In carrying out the process of this invention, typically 150 grams of electrolyte and 15 grams of CaF<sub>2</sub> are charged to the cell in a glove box. The cell is placed within an electric furnace (e.g., Lindberg Model 56622) having a temperature controller (e.g., Lindberg Model 59344) and heated to about 20° C. above the melting point of the electrolyte. During heating about 1 to 2 mol % of the CaF<sub>2</sub> dissolves in the electrolyte, and the remainder forms a layer on the bottom of the crucible. A gas stream comprising 5% by wt fluorine and 95% by wt helium is then bubbled through the melt to remove remaining impurities and to passivate the cell against fluorine to be generated later. Normally the gas stream is bubbled for about 8 hours to insure removal of impurities. The off-gas during passivation can be passed through an activated alumina column to remove fluorine prior to venting.

After passivation, the cell is purged with an inert gas, e.g., argon, to remove residual fluorine. A period of four hours was found to be satisfactory, the absence of fluorine being determined using a KI solution. After purging, the cathode metal pieces are added to the cell under a fast argon flow. Temperature can be monitored by providing a well 34 suitable for placing a thermocouple therein. Once the cathode is molten, the anode and cathode leads can be introduced. In operation, the molten cathode metal pool partially covers the undissolved CaF<sub>2</sub>. The anode and cathode leads are then connected to a potentiostat-galvanostat (e.g., Princeton Applied Research Model No. 173) which is equipped with a function generator (e.g., Princeton Applied Research Model 175). Cell voltage can be recorded on a multimeter (e.g., Keithley Model 616), and transients can be recorded on a digital storage oscilloscope (e.g., Nicolet Model No. 2090).

Located downstream from the cell is a trap for BF<sub>3</sub> (or CaF<sub>2</sub> or LiF) followed by a KI solution in which I<sub>2</sub> is formed by reaction with fluorine generated during electrolysis. The trap and KI solution were also purged with an inert gas prior to operation to remove impurities, and the KI solution was protected from air oxidation by a bubbler filled with silicone oil.

In the electrolysis of CaF<sub>2</sub> solutions in molten salts the evolution of fluorine on the anode is accompanied by deposition of a metal from the electrolyte at the cathode. The potentials at which the cations K, Ca, Na, and Li may be discharged are very close, but deposition can be influenced by operating variables. Consequently, determination of decomposition potentials at these cations at operating conditions is of practical importance for the selection of an optimum operating current density range. Cell voltages (E) were measured as a function of applied constant current (I) at increasing anode current densities between 0 and 100 mA/cm<sup>2</sup>. Plots of E vs. I produced plateaus where E remains constant although I is being increased. Such plateaus, when extrapolated to a zero current density, indicate the voltage at which the cation is being reduced. The plateau region, therefore, is a preferred operating region for the electrolysis.

Voltage vs. current measurements were made for three tetrafluoroborate containing electrolytes: For LiBF<sub>4</sub>/LiF (90/10 mol %) at 315° C., for LiBF<sub>4</sub>/NaBF<sub>4</sub> (50/50 mol %) at 340° C., and for NaBF<sub>4</sub>/KF (90/10 mol %) at 375° C. first plateau in the E vs. I plot occurred at 1.45 volts for all three eutectics (when extrapolated to I=0). This indicated the decomposition of an impurity common to all three eutectics, e.g., water.

The LiBF<sub>4</sub>/LiF eutectic showed a plateau between 45 and 80 mA/cm<sup>2</sup> at 3.9 volts; the same eutectic with CaF<sub>2</sub> dissolved in it exhibited an additional plateau between 35 and 40 mA/cm<sup>2</sup> at 3.45 volts. Hence, the reduction of Li<sup>+</sup> would be expected at 3.9 V and the reduction of Ca<sup>2+</sup> would be expected at 3.45 V. To minimize reduction of Li<sup>+</sup> a current density of 45 mA/cm<sup>2</sup> was used.

The LiBF<sub>4</sub>/NaBF<sub>4</sub> melt with and without CaF<sub>2</sub> dissolved in it exhibited plateaus between 35 to 100 mA/cm<sup>2</sup> which, when extrapolated to I=0, intersected at 3.45 V and 3.9 V. This indicated that the reduction of Na<sup>+</sup> occurs at the same potential, namely 3.45 V, as does the reduction of Ca<sup>2+</sup> at current densities of 35 to 40 mA/cm<sup>2</sup>.

For NaBF<sub>4</sub>/KF with CaF<sub>2</sub> dissolved in it, the first significant plateau occurred at 3.0 volts between 0 to 40 mA/cm<sup>2</sup>. This corresponds to K<sup>+</sup> reduction. A second plateau occurred at 3.45 volts between 40 to 70 mA/cm<sup>2</sup>, and this corresponds to codeposition of Na and Ca.

Thus, codeposition of Ca and alkali metals is unavoidable when electrolyzing CaF<sub>2</sub> in the presence of a large excess of tetrafluoroborate salts of alkali metals whose decomposition potentials are close to that of Ca<sup>2+</sup>. Li based electrolytes offer an electrochemical advantage for a cleaner Ca deposit since the difference in decomposition potentials between Ca<sup>2+</sup> and Li<sup>+</sup> is greater than the difference between Ca<sup>2+</sup> and the other alkali metal based electrolytes. Li salts, however, are known to be more expensive than the Na or K analogs.

In practicing the process of this invention it is possible to minimize the concentration of codepositing alkali metals by selecting as the cathode a Sn/Zn alloy. Zn exhibits preferential solubility for Ca over the alkali metals and the Sn/Zn alloy has an operating temperature below 400° C. It is contemplated that any zinc alloy which is selective for Ca may be used as the cathode material as well as other metals which alloy with Ca but not with any or all other alkali metals.

The electrochemical processes involved in practicing the present invention involve at the cathode:



and



where M=Li, Na, or K.

At the anode fluorine can evolve according to:



as well as according to:



A large excess of BF<sub>4</sub><sup>-</sup> present during electrolysis at the anode should make the latter a predominant path.

Consequently, the overall reactions which occur are as follows:



The practice of the present invention provides further for the removal of  $\text{BF}_3$  from the anode off-gas by absorption on  $\text{CaF}_2$  or any of the alkali metal fluorides according to the following equation:



or



which yields an anode gas free of  $\text{BF}_3$  and allows for recycling of the  $\text{BF}_4^-$  salt thus produced.

The present invention is illustrated in more detail in the following examples wherein anode current efficiency (ACE) is the ratio, in percent, of the quantity of fluorine actually produced to the quantity of fluorine which could be produced theoretically by the number of coulombs passed, and cathode current efficiency (CCE) is the ratio of metals actually produced to the theoretically possible amount of metals which could have been produced. ACE was determined by measuring the amount of iodine formed in a KI solution by reaction of fluorine generated during electrolysis. CCE was determined by dissolving the cathode in acid and determining Na, K, Li, and Ca by atomic absorption spectroscopy.

Positive identification of  $\text{BF}_3$  was made by IR spectroscopy using the intense  $\text{BF}_3$  bands at 1504, 1452, 721, 693, and 480  $\text{cm}^{-1}$ . In all of the examples there was no IR evidence that significant amounts of fluorocarbons were formed during electrolysis.

#### EXAMPLE 1

This Example shows that electrolysis of  $\text{CaF}_2$  dissolved in a  $\text{NaBF}_4/\text{KF}$  eutectic at 375° C. produces fluorine at the anode and that the preferred anode material is pyrolytic graphite.

A solution of 1 mol % of  $\text{CaF}_2$  in 90 mol %  $\text{NaBF}_4$  and 10 mol % KF was electrolyzed between a pool of molten lead (200 grams) as the cathode and anodes consisting of nickel, graphite, pyrolytic graphite and glassy carbon. During the electrolysis the anode gases were flushed from the cell with a stream of argon into a 3 M KI solution. Upon initiation of the electrolysis, the KI solution became yellow and then brownish-red after passage of 8000 coulombs. In the case of the graphite electrode analysis of the KI solution for  $\text{I}_2$  showed that the anode current efficiency (ACE) had been 23.1%.

Visual inspection showed severe corrosion of the Ni anode. Of the carbon anodes tested, pyrolytic graphite and glassy carbon showed less attack than graphite. Pyrolytic graphite was used as the anode material for subsequent experiments for economy.

#### EXAMPLE 2

This Example shows that fluorine is evolved at the anode at current densities of 20 to 200  $\text{mA/cm}^2$  at cell voltages of 2.8 to 16.3 volts and that  $\text{BF}_3$  is evolved along with  $\text{F}_2$  at the anode.

The procedure in Example 1 was repeated at different current densities; the anode was pyrolytic graphite, the

cathode was lead. Current densities (CD) and the corresponding anode current efficiencies (ACE) and cell voltages (CV) are listed in Table I.

TABLE I

|   | CD<br>[mA/cm <sup>2</sup> ] | ACE<br>[%] | CV<br>[volts] |
|---|-----------------------------|------------|---------------|
| 5 | 200                         | 12.2       | 16.3          |
|   | 80                          | 23.1       | 8.6           |
|   | 40                          | 29.5       | 5.0           |
|   | 20                          | 16.4       | 2.8           |

The highest ACE was achieved at a CD of 40  $\text{mA/cm}^2$ .

15 In addition to  $\text{F}_2$ , a white fog appeared in the trap above the KI solution, and a white solid precipitated at the bottom of the trap. This precipitate contained boron and fluorine in a molar ratio of 1:3 and was the hydrolysis product of  $\text{BF}_3$ . The presence of  $\text{BF}_3$  in the anode off-gas was established independently by IR spectroscopy: the dominant bands in the sample spectrum at 1504, 1452, 721, 693 and 480  $\text{cm}^{-1}$  were those of  $\text{BF}_3$ .

#### EXAMPLE 3

This Example shows a  $\text{LiBF}_4/\text{LiF}$  eutectic as the solvent for  $\text{CaF}_2$ .

15 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050

BF<sub>3</sub> occurred after passage of 32,000 coulombs which corresponded to a 70% conversion of LiF to LiBF<sub>4</sub>.

I claim:

1. A process for producing fluorine from calcium fluoride comprising:

(a) dissolving calcium fluoride in a molten salt electrolyte containing an alkali tetrafluoroborate; and  
 (b) electrolyzing the electrolyte at a temperature below 400° C. between an anode selected from a carbon material and nickel and a cathode selected from lead, tin, zinc, and tin/zinc alloy.

2. The process of claim 1 wherein the anode is a carbon material selected from pyrolytic carbon and

glassy carbon and the cathode is a tin/zinc alloy containing 80 mol % tin.

3. The process of claim 1 or claim 2 wherein the electrolyte contains one or more alkali metal fluorides or mixtures thereof wherein the alkali metals are selected from sodium, potassium, and lithium.

4. The process of claim 3 wherein the electrolyte has the composition LiBF<sub>4</sub>/LiF, 90/10 mol %.

5. The process of claim 3 wherein the electrolyte has the composition LiBF<sub>4</sub>/NaBF<sub>4</sub>, 50/50 mol %.

6. The process of claim 3 wherein the electrolyte has the composition NaBF<sub>4</sub>/KF, 90/10 mol %.

\* \* \* \* \*

15

20

25

30

35

40

45

50

55

60

65